

March 1, 1960

G. A. MARSH ET AL

2,927,068

INHIBITING CORROSION

Filed Dec. 23, 1957



INVENTORS.

BY GLENN A. MARSH  
EDWARD SCHASCHI

*Edward A. Schashi*  
ATTORNEY

# United States Patent Office

2,927,068

Patented Mar. 1, 1960

1

2,927,068

## INHIBITING CORROSION

Glenn A. Marsh and Edward Schaschl, Crystal Lake, Ill., assignors to The Pure Oil Company, Chicago, Ill., a corporation of Ohio

Application December 23, 1957, Serial No. 704,818

7 Claims. (Cl. 204—147)

This invention relates to cathodic protection of ferrous metal structures submerged under water or buried underground, and is more particularly directed to a method of treating such structures prior to submerging or burying them in order to reduce the amount of current necessary to give adequate cathodic protection against corrosion.

It is common practice to apply cathodic protection to structures such as pipe lines buried underground or submerged under water, as well as to structures such as drilling platforms erected in water and ships used in salt water. It is also common practice to wrap, coat or encase ferrous metal structures which are buried or submerged in order to prevent corrosion. Such methods are expensive. Where coating or wrapping is not practiced, the amount of current required to afford necessary cathodic protection is usually prohibitive.

We have discovered an inexpensive method of treating such structures prior to burying underground or submerged in water which is inexpensive and enables adequate cathodic protection to be obtained with approximately 2-20% of the current which is ordinarily required for uncoated structures.

Our invention resides in coating the surface with a solution of an alkali metal hexametaphosphate, drying the coating, and then applying a second coating of a solution of an alkali metal chromate or dichromate and a phosphoric acid, and drying the second coating prior to submerging or burying the pipe.

It is an object of our invention to provide an inexpensive method for protecting ferrous metal structures buried underground or submerged under water against corrosion. It is another object of our invention to provide an inexpensive coating on ferrous metal structures which will enable buried or submerged structures to be cathodically protected against corrosion by a small amount of current. Other objects of the invention will become manifest from the following description and the accompanying drawing, of which the single figure is a graph showing rate of corrosion of test specimens when protected in accordance with this invention as compared with specimens which are not so protected.

In accordance with our invention, the structure to be protected, such as pipe or piling, is wire-brushed or sanded to remove loose rust, and then degreased by scrubbing with carbon tetrachloride or equivalent grease solvent. The clean structure is then coated with a solution, preferably freshly prepared, of an alkali metal hexametaphosphate, preferably sodium hexametaphosphate. A solution of any desired concentration may be used but we prefer a solution of about 5-20% by weight sodium hexametaphosphate. The solution is applied to the structure by brushing, spraying, dipping, or any other suitable manner. Where the coating is performed by dipping or immersing, the specimen may be left in the solution for a period of 1-100 minutes at a temperature of about 40-120° F. We prefer to maintain the solution at about 60-90° F. and allow the structure to re-

2

main immersed for about 5-15 minutes, after which it is dried in air and then given a second coating with a solution of an alkali metal chromate or dichromate, such as sodium or potassium dichromate, containing a phosphoric acid, such as meta-, ortho-, or pyro-phosphoric acid. We prefer to use a dilute, aqueous solution containing about 0.5-1% of sodium dichromate and in the neighborhood of about 0.1-1% of phosphoric acid. Dilute solutions should be used so that when the coating is dried it will be very thin, weighing less than 1 gram per sq. ft. In coating with the dichromate-phosphoric acid solution the temperature of the solution should be maintained at about 40-120° F., and where immersion is used, the period of immersion will be about 1-100 minutes. Preferred conditions of immersion are 90-120° F. for a period of 5-10 minutes.

Where the structure to be protected is one which is partially corroded or rusted, it has been found expedient to repeat the hexametaphosphate coating after coating with the dichromate-phosphoric acid solution, and drying, and to also repeat the dichromate-phosphoric acid coating after the second hexametaphosphate coating and drying. Where the structure to be protected is clean, only a single coating with the hexametaphosphate and with the dichromate-phosphoric acid solution is required.

In order to demonstrate the invention, an ordinary rusted steel specimen was wire-brushed to remove loose rust and then degreased by scrubbing with carbon tetrachloride. The degreased specimen was immersed for 15 minutes at room temperature in a freshly prepared 20% solution of hexametaphosphate, after which it was removed, drained and allowed to dry in air. After the specimen was dried it was immersed for 10 minutes in an aqueous solution at 120° F., containing 0.67% by weight of sodium dichromate and 0.5% by weight of 85% phosphoric acid. The specimen was removed from the second solution, drained, and dried in air. The treatment just described with the two solutions was repeated on the specimen, after which the specimen was immersed in aerated, agitated water and cathodic protection was applied at a current density of 3 milliamperes per sq. ft. of surface area. No visible corrosion occurred over a period of a 30-day test period.

In order to further demonstrate the efficacy of the method constituting our invention, a series of experiments were performed, the results of which are graphically represented in the drawing. In these tests corrosion test-probes of the type similar to those sold by Labline, Inc. and disclosed in their Bulletins Nos. 52 and 5205, and claimed in our copending application Serial No. 528,032, filed August 12, 1955 and also in application of Lynn E. Ellison, Serial No. 631,697, filed December 31, 1956, Patent No. 2,824,283, in which the test element was made of mild steel, were used in the tests, and loss of thickness was read directly on the corrosion meter. The results in these tests are shown in the drawing by plotting a loss in thickness in micro-inches against time. The slope of the curve at any point is the corrosion rate at that particular time. Curve A represents the results obtained using a probe which had been coated in the manner just described in connection with the previous example, but to which no cathodic protection was applied. Curve B shows the results obtained with a probe which had not been coated but to which a cathodic protection of 1 ma./sq. ft. current density had been applied. Curve C shows the results obtained when the probe was coated in the manner described in connection with the previous example and to which cathodic protection current had been applied at a current density of 1 ma./sq. ft. In this test the current was interrupted for one hour during each 24 hours. In a similar test, represented by curve D, the current was applied continuously without interruption. The results

as depicted in the drawing show that not only does the combination of coating and low current-density cathodic protection afford substantially complete protection against corrosion, but, it further shows that interruption of the current does not have a serious detrimental effect on the protection afforded. Maximum protection is obtained, however, when the current is continuous.

A further series of tests was run to determine whether other solutions when used in conjunction with low-density cathodic current would protect rusted steel against corrosion. The various solutions used in these tests and the combinations in which the solutions were used for coating the probes are given in the following Tables I and II.

TABLE I  
*Solutions used in tests*

| Identification No. | Composition                                                                                                                                                                                              |
|--------------------|----------------------------------------------------------------------------------------------------------------------------------------------------------------------------------------------------------|
| A                  | 50% $H_3PO_4$ —50% Formula 30 alcohol.                                                                                                                                                                   |
| B                  | 10% NaOH.                                                                                                                                                                                                |
| C                  | 5% Chromic Acid.                                                                                                                                                                                         |
| D                  | 10% Chromic Acid.                                                                                                                                                                                        |
| E                  | Conc. $HNO_3$ .                                                                                                                                                                                          |
| F                  | 30% $HNO_3$ .                                                                                                                                                                                            |
| G                  | 2% Versene Fe-3.                                                                                                                                                                                         |
| H                  | 5% Sodium Hexametaphosphate.                                                                                                                                                                             |
| I                  | 20% Sodium Hexametaphosphate.                                                                                                                                                                            |
| 1                  | Straight $H_3PO_4$ .                                                                                                                                                                                     |
| 2                  | 50-50 $H_3PO_4$ +Formula 30 alcohol.                                                                                                                                                                     |
| 3                  | 20% Sodium Hydroxide.                                                                                                                                                                                    |
| 4                  | 20% Sodium Hydroxide saturated in Sodium Nitrite.                                                                                                                                                        |
| 5                  | Water Glass.                                                                                                                                                                                             |
| 6                  | Water Glass 90%+Calcium Chloride 10% plus 500 g. dist. water.                                                                                                                                            |
| 7                  | Saturated sodium chromate.                                                                                                                                                                               |
| 8                  | 50-50 Sat'd. potassium dichromate— $H_3PO_4$ .                                                                                                                                                           |
| 9                  | Saturated potassium dichromate solution, 500 cc.+1 cc. sulfuric acid.                                                                                                                                    |
| 10                 | 50-50 Phosphoric acid+distilled water plus 10 g. iron filings.                                                                                                                                           |
| 11                 | 50-50 $H_3PO_4$ +Formula 30 alcohol (added 10 g. manganese sulfate).                                                                                                                                     |
| 12                 | 50-50 Phosphoric acid+water solution (to 200 cc. of this added zinc granules until just saturated with zinc, then added 20 cc. phosphoric acid).                                                         |
| 13                 | 350 g.—350 g. Phosphoric acid+ $H_2O$ (added iron filings in excess, after bubbles stopped; filtered through coarse filter paper; added 100 cc. of $H_3PO_4$ ; then added 10 cc. of manganese chloride). |
| 14                 | 250 g.—250 g. $H_3PO_4$ +water (added zinc granules in excess, after bubbles stopped; poured off the solution leaving zinc behind. Then added 50 cc. $H_3PO_4$ . Then added 10 cc. manganese chloride).  |
| 15                 | Saturated Calcium Chloride+5% $H_3PO_4$ .                                                                                                                                                                |
| 15B                | 5% Tri-Sodium Phosphate.                                                                                                                                                                                 |
| 16                 | 10% Potassium Permanganate.                                                                                                                                                                              |
| 17                 | 5% Ammonium Persulfate.                                                                                                                                                                                  |
| 18                 | 50-50 (20% Sodium Hydroxide saturated with Sodium Nitrite)—water glass.                                                                                                                                  |
| 19                 | 50% Water Glass.                                                                                                                                                                                         |
| 20                 | 50% NaOH.                                                                                                                                                                                                |
| 21                 | 50% Water Glass—5% (20% NaOH) 45% water.                                                                                                                                                                 |
| 22                 | 5% Water Glass—95% (20% NaOH).                                                                                                                                                                           |
| 23                 | 5% Water Glass, 45% (20% NaOH) 50% water.                                                                                                                                                                |
| 24                 | 20% Calcium Chloride.                                                                                                                                                                                    |
| 25                 | 10% Copper Sulfate.                                                                                                                                                                                      |
| 26                 | Mercuric Nitrate.                                                                                                                                                                                        |
| 27                 | 5% Sodium Arsenite.                                                                                                                                                                                      |
| 28                 | Saturated Sodium Chromate.                                                                                                                                                                               |
| 29                 | Saturated sodium bicarbonate.                                                                                                                                                                            |
| 30                 | 0.67% Sodium Dichromate.                                                                                                                                                                                 |
| 31                 | 0.5% Phosphoric Acid.                                                                                                                                                                                    |
| 32                 | 98.53% Water.                                                                                                                                                                                            |
| 33                 | 0.2% Sodium Nitrite.                                                                                                                                                                                     |
| 34                 | 0.2% Diammonium Hydrogen Phosphate.                                                                                                                                                                      |
| 35                 | 99.6% Water.                                                                                                                                                                                             |
| 36                 | 0.5 Sodium Nitrite.                                                                                                                                                                                      |
| 37                 | 0.5% Diammonium Hydrogen Phosphate.                                                                                                                                                                      |
| 38                 | 99.6% Water.                                                                                                                                                                                             |
| 39                 | 0.5% Sodium Nitrite.                                                                                                                                                                                     |
| 40                 | 0.25% Disodium Phosphate.                                                                                                                                                                                |
|                    | 0.25% Monosodium Phosphate.                                                                                                                                                                              |
|                    | 99.00% Water.                                                                                                                                                                                            |
|                    | 0.5% Sodium Nitrite.                                                                                                                                                                                     |
|                    | 0.37% Disodium Phosphate.                                                                                                                                                                                |
|                    | 0.13% Monosodium Phosphate.                                                                                                                                                                              |
|                    | 99.00% Water.                                                                                                                                                                                            |
|                    | Saturated Trisodium phosphate.                                                                                                                                                                           |
|                    | Sodium Nitrite 0.5%.                                                                                                                                                                                     |
|                    | 0.5% Diammonium Phosphate.                                                                                                                                                                               |
|                    | 0.5% Sodium Nitrite.                                                                                                                                                                                     |
|                    | 0.5% Diammonium Phosphate.                                                                                                                                                                               |
|                    | 99.00% Water.                                                                                                                                                                                            |
|                    | 0.5% Sodium Nitrite.                                                                                                                                                                                     |
|                    | 0.5% Disodium Phosphate.                                                                                                                                                                                 |
|                    | 0.1% Monosodium Phosphate.                                                                                                                                                                               |
|                    | 99.00% Water.                                                                                                                                                                                            |

15 TABLE II  
*Solution applied as coating and order in which applied to test specimen*

|    | First Coating | Second Coating | Third Coating | Fourth Coating |
|----|---------------|----------------|---------------|----------------|
| 20 |               |                |               |                |
|    | A             | 30             |               |                |
|    | A             | 21             |               |                |
|    | A             | 26             |               |                |
|    | A             | 27             |               |                |
| 25 | A             | 26             | 27            | 21             |
|    | A             | 30             | 21            |                |
|    | A             | 26             | 21            |                |
|    | A             | 27             | 21            |                |
|    | A             | 36             |               |                |
|    | A             | 37             |               |                |
|    | A             | 39             |               |                |
|    | A             | 40             |               |                |
| 30 | A             | 41             |               |                |
|    | A             | 42             |               |                |
|    | A             | 37             | 38            |                |
|    | A             | 39             | 36            |                |
|    | A             | 40             | 36            |                |
|    | A             | 41             | 36            |                |
|    | A             | 39             | 36            |                |
|    | A             | 36             | 37            |                |
| 35 | A             | 39             | 27            |                |
|    | A             | 40             | 27            |                |
|    | A             | 41             | 27            |                |
|    | A             | 39             | 36            | 27             |
|    | A             | 40             | 36            | 27             |
|    | A             | 41             | 36            | 27             |
|    | A             | 42             | 36            |                |
| 40 | A             | 42             | 27            |                |
|    | A             | 42             | 36            | 27             |
|    | A             | 43             |               |                |
|    | A             | 43             |               |                |
|    | A             | 44             |               |                |
|    | A             | 45             |               |                |
|    | A             | 37             | 30            |                |
|    | A             | 37             | 30            | 26             |
| 45 | A             | 30             | 37            |                |
|    | A             | 30             | 37            | 26             |
|    | A             | 26             | 37            |                |
|    | A             | 26             | 37            |                |
|    | A             | 37             | 26            |                |
|    | A             | 30             | 26            |                |
|    | A             | 37             | 26            | 30             |
|    | A             | 30             | 26            | 37             |
| 50 | A             | 26             | 30            |                |
|    | A             | 26             | 30            | 37             |
|    | A             | 26             | 5             |                |
|    | A             | 26             | 27            |                |
|    | A             | 26             | 27            | 5              |
|    | A             | 27             | 26            | 5              |
|    | A             | 27             | 26            | 21             |
| 55 | A             | 3              | 5             |                |
|    | A             | 29             |               |                |
|    | A             | 29             | 5             |                |
|    | A             | 30             | 5             |                |
|    | B             | 30             |               |                |
|    | C             | 30             |               |                |
|    | D             | 30             |               |                |
|    | E             | 30             |               |                |
|    | F             | 30             |               |                |
|    | G             | 30             |               |                |
|    | H             | 30             |               |                |
|    | I             | 30             |               |                |

In no case were the solutions effective in affording protection except in the two tests in which the probe was initially coated with the sodium hexametaphosphate solution and then coated with the sodium dichromate-phosphoric acid solution.

Our invention is equally effective in protecting hot-  
70 rolled and cold rolled steel and in protecting other fer-  
rous metal alloys.

The coatings are easy and inexpensive to apply, it being necessary only to coat the entire surface to be protected and permit each coating to dry before applying the subsequent coating or before immersing or burying

the structure. Whereas it is often necessary to use in the neighborhood of 30-50 ma./sq. ft. current density to protect uncoated structures, we are able to fully protect structures which have been coated in accordance with our invention by the application of as little as 1 ma./sq. ft. of current density. In applying our invention to a structure to be protected, we prefer after burying or submerging the structure to initially apply a higher current density of the order of 10-20 ma./sq. ft. and gradually decrease the current density to the minimum required to afford protection as indicated by corrosion-meter tests.

What is claimed is:

1. In a process for cathodically protecting ferrous metal structures, submerged in water or buried beneath the ground, against corrosion, the steps of coating the bare metal structure with a solution of alkali metal hexametaphosphate, drying the coating, then coating the structure with a second solution containing a phosphoric acid and an alkali metal salt of the group consisting of alkali metal chromates and dichromates, drying the coating before submerging or burying the structure, contacting said coating with the water or ground, and cathodically protecting the structure by applying thereto a current having a density equal to a small fraction of that required to protect the uncoated structure against corrosion.

2. Process in accordance with claim 1 in which the structure is cleaned and degreased prior to applying the solution of alkali metal hexametaphosphate thereto.

30

3. Process in accordance with claim 2 in which the alkali metal hexametaphosphate is sodium hexametaphosphate.

5 4. Process in accordance with claim 3 in which the second solution is a dilute solution of phosphoric acid and sodium dichromate.

10 5. Process in accordance with claim 4 in which the sodium hexametaphosphate is an aqueous solution containing 5-20% of sodium hexametaphosphate and the second solution is an aqueous solution containing about 0.67% sodium dichromate and about 0.5% phosphoric acid by weight.

6. A process according to claim 1 in which the current density is about 1 milli-ampere per square foot.

15 7. A process according to claim 1 in which the current density is initially 10-20 milli-amperes per square foot and is gradually decreased to the minimum current density required to afford substantially complete cathodic protection as indicated by corrosion rate measurements.

References Cited in the file of this patent

UNITED STATES PATENTS

|    |           |                    |               |
|----|-----------|--------------------|---------------|
| 25 | 2,163,984 | Pekovic            | June 27, 1939 |
|    | 2,337,856 | Rice               | Dec. 28, 1943 |
|    | 2,499,261 | Rosenbloom         | Feb. 28, 1950 |
|    | 2,787,557 | Christensen et al. | Apr. 2, 1957  |